

## UNITED STATES PATENT OFFICE

2,560,151

METHOD OF COATING ELECTRICAL  
CONTACT PINS

Anna Margareta Bergö-Heineman, Stockholm,  
Sweden, assignor to Aktiebolaget Svenska Elek-  
tronror, Stockholm, Sweden, a corporation of  
Sweden

No Drawing. Application February 14, 1947, Se-  
rial No. 728,732. In Sweden December 23,  
1944

Section 1, Public Law 690, August 8, 1946  
Patent expires December 23, 1964

2 Claims. (Cl. 117—130)

1

The present invention relates to a method for obtaining electrically well-conducting surfaces on contacting members and has been developed to improve the electrical conductivity of contact pins and the like of chrome-iron alloys for electrical discharge tubes, said contacting members becoming deteriorated by oxidation, for example, during some process in the manufacture of the tube so that undesirable changes and irregularities appear in the conductivity of the contact surface.

In the manufacture of radio tubes of the so-called press-moulded glass type, the contact pins usually consist of chrome-iron wires which during the compression of the base plate or the tube are sealed into the glass mass of the plate. In connection with the press moulding of the base plate the contact pins are subjected to a certain oxidation resulting in a considerable fluctuation of the contacting properties between pins of different tubes. Normally the oxide contaminants are eliminated by reduction by means of the flames sweeping the tube during its manufacture, but chrome oxide is not removed so easily. According to the invention, this inconvenience is overcome in such a manner that when the electrode system of the tube has been mounted on the base plate with its contact pins, the contact pins are covered, prior to the sealing of the tubular envelope, with zapon lacquer in which silver oxide has been suspended. In connection with the sealing of the envelope with the base plate the lacquer is burnt away and the silver oxide is reduced to metal. Probably the conversion of the silver oxide is a repeated process, the reduced silver reacting with the oxygen in the chrome oxide on the contact pins into silver oxide which again is dissociated into metallic silver etc. This effect of the silver oxide which in this connection may be considered essentially active as an autocatalyzer for the disintegration of the chrome oxide coating of the contact pins, results in the production of smooth bright contact pins of good contacting properties.

In some cases, however, certain difficulties may appear in getting the metal obtained by the heating of the compound to sinter sufficiently firmly together with the base especially if the thermal dissociation of the compound is effected at too low a temperature respectively if the base is covered with a relatively strong oxide coating. It is proved, however, that a very good adhesion

2

may be obtained by providing the compound dissociable into metal with an addition of lead borate. Bright contact surfaces can be produced by using a suspension of 3—25, preferably 8—15, parts by weight of silver oxide to one part by weight of lead borate (lead metaborate) in a suspender such as ethylene glycol or some other suitable medium, giving the whole a greasy condition for coating the contact surfaces. In the treatment of contact pins for discharge tubes very satisfactory results have been obtained with a coating mixture with the composition

20 parts by weight of silver oxide  
15 2.5 parts by weight of lead metaborate  
21 21 parts by weight of ethylene glycol.

For the preparation of the mixture the silver oxide was first ground in a ball mill for 24 hours, the silver oxide so treated then being ground 20 in a mortar together with the lead borate until they were well mixed, whereupon ethylene glycol is added and a further grinding during a short time is performed. The contact pins are coated 25 with the paste before the sealing of the stem with the tubular envelope.

The lead borate insures that the covering paste firmly sinters together with the base and that the well adhering layer shows a very good electrical conductivity on account of its great content of silver.

What I claim is:

1. The method of producing a surface having good electrical conducting characteristics on contact pins of a chrome-iron alloy sealed in electrical lamp bases by dissociating the chrome oxide layer formed on said pins when said bases are sealed which includes the steps of applying a silver oxide coating to the surfaces of said pins having said chromium oxide layer thereon and applying heat to said coating sufficient to dissociate said silver oxide to silver, to cause said silver to react with the chromium oxide to dissociate same, and to sinter the residual silver onto the surfaces of said contact pins.

2. The method as set forth in claim 1 which includes the additional step of mixing said silver oxide with a lead borate flux prior to application to said contact pins.

50 ANNA MARGARETA BERGÖ-HEINEMAN.

(References on following page)

## REFERENCES CITED

The following references are of record in the file of this patent:

## UNITED STATES PATENTS

| Number    | Name   | Date          |
|-----------|--------|---------------|
| 1,922,387 | Muller | Aug. 15, 1933 |
| 1,977,625 | Ernst  | Oct. 23, 1934 |

| Number    |
|-----------|
| 1,999,529 |
| 2,429,088 |

| Name  | Date          |
|-------|---------------|
| Smith | Apr. 30, 1935 |
| Box   | Oct. 14, 1947 |

## FOREIGN PATENTS

| Country       | Date          |
|---------------|---------------|
| Great Britain | Mar. 22, 1934 |
| Sweden        | Oct. 12, 1948 |